

1

2,824,836

## LUBRICATING OIL COMPOSITIONS

Harlan M. Smith, Roselle, William Hoerner, Linden, and James R. Davidson, Iselin, N. J., assignors to Esso Research and Engineering Company, a corporation of Delaware

No Drawing. Application November 1, 1954  
Serial No. 466,196

4 Claims. (Cl. 252—32.7)

This invention relates to lubricants and more particularly relates to lubricating oil compositions useful as crankcase lubricants for internal combustion engines and to addition agents for such compositions which reduce the wear of engine parts.

The utilization of additives in lubricating oil compositions is well known. Such additives have been used to improve various characteristics of lubricating oil base stocks such as viscosity index, pour point, odor, corrosivity, oiliness, film strength, detergency, etc. The need for improved lubricating oil additives continues to increase as the severity of engine operation becomes greater. It has recently been found that conventional lubricating oil compositions have been deficient in preventing wear of certain engine parts, particularly in high horsepower output V-8 engines. This wear of engine parts has occurred particularly in the valve gear or train of these V-type engines. More specifically, difficulties have been encountered with the cam lobes, cam followers and rocker arms in these valve trains. Valve train wear is particularly severe with overhead valve V-8 engines. Wear on lobes of camshafts and on faces of cam followers is the most serious type of wear. In an advanced stage it can cause noisy operation, less efficient engine operation due to the fact that valves are opened less widely, and in an extreme stage the valves do not open widely enough to permit operation at all. There has thus been a critical need for lubricating oil compositions which, in addition to having the conventionally desirable properties of detergency, viscosity index and the like, also will reduce the wear of engine parts.

It has now been found that esters derived from ricinoleic acid are exceedingly effective in reducing such valve train wear. It has also been found that a combination of these esters and zinc dialkyl dithiophosphates is even more effective than the individual materials themselves in reducing valve train wear. More specifically, the improved lubricating oil compositions of this invention comprise a major proportion of a lubricating oil base stock, in the range of about 0.05 to 2.5% by weight, based on the total composition, of a zinc dialkyl dithiophosphate having in the range of about 3 to 20 carbon atoms in each alkyl group, and in the range of about 0.1 to 1.5% by weight, based on the total composition, of an ester derived from ricinoleic acid. Preferred lubricating oil compositions of this invention also contain in the range of about 0.5 to 15% by weight, based on the total composition, of a detergent selected from the group consisting of alkaline earth metal alkyl phenol sulfides, alkaline earth metal sulfonates and mixtures thereof. Other preferred compositions also include viscosity index improvers such as olefin polymers and ester polymers.

The zinc dialkyl dithiophosphates of this invention have the following formula



2

where R is an alkyl group of about 3 to 20 carbon atoms. The two R radicals in the above formula may be different alkyl groups. The preferred zinc compounds are those containing in the range of about 8 to 16 carbon atoms per molecule, preferably those containing about 12 carbon atoms per molecule. Specific examples of these zinc dialkyl dithiophosphates include zinc dibutyl dithiophosphate, zinc propyl octyl dithiophosphate, zinc isopropyl hexyl dithiophosphate, zinc isopropyl 2-ethylhexyl dithiophosphate, zinc amyl methylcyclohexyl dithiophosphate and the like.

The preparation of these zinc compounds is well known in the art and is based on the following reactions:



The zinc dialkyl dithiophosphates are preferably prepared by reacting the alcohols, or alcohol mixtures, with phosphorus pentasulfide preferably in the ratio of about 1 mole of  $P_2S_5$  to about 4 moles of the alcohol. This reaction is preferably carried out with agitation at an elevated temperature in the range of about 165° to 215° F. in the presence or absence of a solvent until the evolution of hydrogen sulfide substantially ceases. The zinc salts are then produced from the free dithiophosphoric acid esters so obtained by introducing approximately the theoretical quantity of zinc or zinc oxide with agitation at about 120° to 210° F. until a solution of the zinc salt is obtained. Alternatively, the alkali metal salts of the dithiophosphoric acid esters may be formed initially by neutralization with alkali carbonates or hydroxides and subsequently these alkali metal salts may be converted to the corresponding zinc dithiophosphates by double decomposition with an aqueous solution of a zinc salt.

The alcohols utilized in the preparation of the zinc dialkyl dithiophosphates of this invention are those having about 3 to 20 carbon atoms and are preferably those containing about 3 to 12 carbon atoms per molecule. As examples of these alcohols may be mentioned propyl, isopropyl, butyl, isobutyl, amyl, isoamyl, iso-hexyl, n-octyl, iso-octyl, 2-ethylhexyl, n-decyl, isodecyl, dodecyl, tetradecyl, octadecyl, methylisobutyl carbinol, methyl cyclohexyl, and various alcohols produced from polymers and copolymers of propylene and butylenes via the well-known Oxo reaction. Of the latter may be mentioned specifically the  $C_8$  Oxo alcohol produced from  $C_7$  propylene-butylene dimer, the  $C_{10}$  alcohol produced from tri-propylene, the  $C_{13}$  alcohol produced from tetra-propylene and the  $C_{16}$  alcohol produced from penta-propylene.

The esters useful in this invention are those derived from ricinoleic acid. Acids derived from castor oil by saponification and subsequent acidification may also be employed to form the esters of this invention. These acids derived from castor oil contain about 85% by weight of ricinoleic acid and small amounts of other acids such as oleic, linoleic and stearic acid.

Condensation polymers of ricinoleic acid may also be employed in forming the esters of this invention. These condensation polymers are formed by reacting the carboxylic group of one molecule with the hydroxyl group of another molecule with the elimination of water by a self-esterification reaction. Thus, from 2 up to 6 or more molecules, preferably about 2 to 4 molecules, of ricinoleic acid may be combined to form a condensation polymer.

containing one free carboxylic acid group and one free hydroxyl group. Thus, for example, di-, tri-, tetra-, penta-, and hexa-ricinoleic acid may be formed. The condensation reaction may be carried out simply by heating ricinoleic acid at a temperature above about 210° F. as is well known in the art. This reaction generally forms a mixture of polyricinoleic acids. Such mixtures may be employed in this invention. These condensation polymers may then be esterified to form esters useful in this invention.

The ricinoleic acid esters of this invention are preferably those of glycols or polyglycols which contain in the range of about 2 to 100 carbon atoms per molecule and more preferably are those of glycols or polyglycols which contain in the range of about 2 to 40 carbon atoms per molecule. The preferred glycols contain at least one ether oxygen in the molecule. Thus, polyalkylene glycols, such as polyethylene glycol, polypropylene glycol, polybutylene glycol, and the like, are useful in this invention. The glycols useful in this invention have the general formula



where  $y$  is an integer of 1 to 50, preferably 1 to 20, and  $n$  is an integer of 2 to 4. Specific examples of the glycols useful in this invention include the following:

Ethylene glycol  
Diethylene glycol  
Tetraethylene glycol  
Nonaethylene glycol  
Tetracosaoxyethylene glycol  
Propylene glycol  
Tetrapropylene glycol  
Tetradecapropylene glycol  
Butylene glycol  
Tributylene glycol  
Dodecabutylene glycol

Ricinoleic acid esters of alcohols may also be used in certain instances although these esters are less effective than those formed from glycols or polyglycols. Such alcohols include methyl, propyl, butyl, amyl, octyl, decyl, dodecyl,  $\text{C}_6$  to  $\text{C}_{16}$  Oxo alcohols obtained by the oxonation of  $\text{C}_5$  to  $\text{C}_{15}$  olefins or olefin polymers, alcohols derived from coconut oils, etc.

The esters of this invention are prepared by esterifying ricinoleic acid, castor oil acids (predominantly ricinoleic acid) or polyricinoleic acids with the above-mentioned glycols, polyglycols, alcohols or mixtures thereof by conventional esterification methods, which are well known to the art. A particularly preferred ester useful in this invention is a polyethylene glycol di-ricinoleate, containing a glycol residue having a molecular weight in the range of about 200 to 800, preferably about 400. Other ricinoleates include monoricinoleate-polyethylene glycol pentaricinoleate, diricinoleate polyethylene glycol tetra-ricinoleate and the like.

The alkaline earth metal salts of alkyl phenol sulfides which are utilized in preferred lubricating oil compositions may be obtained by the alkylation of phenol followed by treatment with a sulfur halide and neutralization with an alkaline earth metal base and have the following general formula:



where  $R$  is an alkyl radical containing about 4 to 24 carbon atoms, and preferably about 6 to 12 carbon atoms,  $M$  is an alkaline earth metal and  $x$  is an integer from 1 to 4, preferably 1 to 2. The preparation of these alkaline earth metal salts of phenol sulfides is well known to the art.

Suitable synthetic alkyl phenols for preparing the desired phenol sulfide salts are preferably those containing secondary or tertiary alkyl radicals, because alkylation of phenol occurs more readily with branched chain aliphatic reactants. Commonly, the alkylation reaction involves a condensation of olefins with phenol, the reaction being catalyzed by anhydrous metal halides, boron trifluoride, hydrofluoric acid, stannic chloride with hydrogen chloride, sulfuric acid, phosphoric acid, or certain activated clays. As olefinic reactants, refinery gases containing propylene, butylenes, amylenes, etc., are economically useful, although individual olefins or olefin-containing mixtures derived from other sources may be used. Preferred individual olefins are the butenes, amylenes and olefin polymers, such as tripropylene, diisobutylene or triisobutylene or normal olefin polymers or copolymers of normal and secondary or tertiary olefins or copolymers of olefins and diolefins. The reaction temperature is usually controlled to avoid side reactions. In employing sulfuric acid, a liquid phase reaction at relatively low temperature is preferred, while with phosphoric acid the reaction may be carried out in the vapor phase.

One class of alkyl phenols which are particularly preferred are those which have been prepared by alkylation of phenol with an olefin polymer such as diisobutylene or a refinery butene polymer oil. Alkylation of phenol with about an equal molar proportion of diisobutylene gives p-tert.-octyl phenol, also known as diisobutyl phenol or tetramethyl butyl phenol. This phenolic material is especially desirable because of the ease of its preparation and because products made from it are highly satisfactory for the present invention. In many instances, however, a higher degree of alkylation may be advantageous, and for this reason the phenol may be alkylated with as much as two molecular equivalents of diisobutylene to give, under proper conditions, essentially di-tert.-octyl phenol; or it may be alkylated with other olefin polymers such as triisobutylene or other isobutylene polymers.

Another class of alkyl phenols which are especially preferred are those which are prepared by alkylation of phenol with tripropylene utilizing  $\text{BF}_3$  as a catalyst. Alkylation of phenol with an equal molar proportion of tripropylene gives tripropyl phenol. This phenolic material is also excellent for the purposes of the present invention. In certain instances a higher degree of alkylation may be advantageous and in this case the phenol may be alkylated with as much as two molecular equivalents of tripropylene to give, under proper conditions, essentially di-tripropyl phenol.

Suitable products may also be prepared by alkylating phenol with certain of the polymeric materials obtained as by-products in the manufacture of butyl alcohol from petroleum refinery butenes. These consist essentially of polymers of n-butene with small percentages of isobutene and other olefins and give alkylated phenols having branched chain alkyl groups of 16-20 or 20-24 carbon atoms depending on the polymeric material used in the alkylation. It should be understood that in many cases the alkylation products may be mixtures of various compounds rather than entirely one specific alkyl phenol and that it is intended to use such mixtures in practicing this invention.

For conversion of the alkyl phenol to an alkyl phenol sulfide, the alkyl phenol is reacted with sulfur dichloride to produce essentially a phenol monosulfide having a thioether linkage, while sulfur monochloride may be used to produce essentially the phenol disulfide. About one-half to one mole of sulfur halide is used with each mole of alkyl phenol, and the reaction is preferably carried out in a solvent such as dichlorethane, chloroform, petroleum naptha, benzol, xylol, toluol, and the like. These alkyl phenol sulfides prepared as above may be illustrated by the following general classes of compounds.

## Monosulfides:



## Disulfides:



In the above structural formulas, the alkyl groups contain 4 to 24 carbon atoms and preferably contain 6 to 12 carbon atoms. It will be understood that in the formation of the mono-sulfides and disulfides, small amounts of polysulfides will also be formed. This is even more usually the case where more than the theoretical quantity of sulfur halide is employed in preparing the alkyl phenol sulfide.

For converting the alkyl phenol sulfides to metal salts it is usually sufficient merely to add an alkaline earth metal or an alkaline earth metal oxide, hydroxide, sulfide, alkoxide, hydride or carbide to a mineral oil solution or other solution of the phenol sulfide at an elevated temperature. Thus, barium salts of alkylated phenol sulfides are prepared by reacting the sulfide with barium hydroxide, preferably in the form of the hydrate,  $\text{Ba}(\text{OH})_2 \cdot 8\text{H}_2\text{O}$ . In some instances it may be preferable to prepare these salts from the alkali metal salt by double decomposition. The calcium salts are conveniently prepared by reacting alkyl phenol sulfides with calcium methylate or other calcium alcoholate.

In many cases the metal alkyl phenol sulfide prepared by neutralizing with a metal hydroxide may occur as a hydrated salt. Use of hydrated salts prepared in this manner or by any other method is also contemplated in the present invention. The alkaline earth metal salts include those of calcium, barium, strontium and magnesium, calcium and barium being the preferred metals. Mixtures of salts of different alkaline earth metals may be employed if desired.

The alkaline earth metal sulfonates useful in this invention include those of calcium, barium, strontium and magnesium. The preferred sulfonates are those of calcium and barium. Petroleum sulfonates and particularly the alkaline earth metal soaps of oil soluble or so-called "mahogany" acids which are usually produced during treatment of lubricating oil distillates with concentrated to fuming sulfuric acid are particularly useful in this invention. Such sulfonates are well known to the art and are described, for example, in U. S. Patent No. 2,467,176, etc. The more desirable high molecular weight (350 to 550) acids, particularly those produced when treating white oil with fuming acid, are normally recovered as sodium soaps by neutralizing the acid oil with sodium hydroxide or carbonate, extracting the soaps with aqueous alcohol, distilling off the alcohol and purifying the soap by well-known means from contaminating salts (such as sodium carbonate, sulfate, etc.).

The alkaline earth metal sulfonates may be prepared by direct neutralization of the acid treated oils with an oxide or hydroxide of the desired metal. However, it is

often more convenient to prepare them from the sodium salts by double decomposition. Thus the alkaline earth metal sulfonates may be made by precipitation from alcoholic solution with an alkaline earth metal salt. Or an oil solution of sodium sulfonates may be emulsified with an aqueous solution of the alkaline earth metal salt. For example, the calcium metal sulfonates may be prepared by precipitation from alcohol solution with calcium chloride, the inorganic salts then being removed by washing with water. It will be understood that other sulfonates such as those of alkyl aromatic benzenes, e. g. didodecylbenzene, alkyl naphthalene, etc., may be utilized in this invention. Also, sulfonates prepared by photochemical methods may be employed. Likewise, mixtures of sulfonates of several alkaline earth metals may be used in this invention. The sulfonates are preferably employed in this invention with the alkyl phenol sulfide salts in a ratio of alkyl phenol sulfide salt/sulfonate of about 1:1 to 5:1 on a weight basis.

Preferred compositions also may include a viscosity index improver. The preferred viscosity index additive is a high molecular weight polymerized olefin such as polymerized  $\text{C}_3$  to  $\text{C}_5$  olefins; for example, polymerized butenes, especially polymerized isobutylene having a molecular weight in the range of about 5,000 to 50,000; preferably, about 10,000 to 20,000 are quite useful. These polymerized olefins are readily prepared by procedures well known to the art. Such additives are also useful as thickening agents for increasing the viscosity of relatively light oil base stocks. Other viscosity index improvers include the polymethacrylate esters, fumarate-vinyl acetate copolymers, polyalkyl styrenes, and the like.

The lubricating oil base stocks used in the compositions of this invention may be straight mineral lubricating oils or distillates derived from paraffinic, naphthenic, asphaltic or mixed base crudes, or if desired, various blended oils may be employed as well as residuals, particularly those from which asphaltic constituents have been carefully removed. The oils may be refined by conventional methods using acid, alkali, and/or clay or other agents such as aluminum chloride, or they may be extracted oils produced, for example, by solvent extraction with solvents of the type of phenol, sulfur dioxide, furfural, dichloro ethyl ether, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coal tar fractions and coal tar or shale oil distillates may also be used. Also, for special applications, animal, vegetable or fish oils, or their hydrogenated or volatilized products, may be employed, either alone or in admixture with mineral oils.

Synthetic lubricating oils having a viscosity of at least 30 SSU at 100° F. may also be employed, such as esters of monobasic acids (e. g. ester of  $\text{C}_8$  Oxo alcohol with  $\text{C}_8$  Oxo acid, ester of  $\text{C}_{13}$  Oxo alcohol with octanoic acid, etc.), esters of dibasic acids (e. g. di-2-ethyl hexyl sebacate, di-nonyl adipate, etc.), esters of glycols (e. g.  $\text{C}_{13}$  acid diester of tetraethylene glycol, etc.), complex esters (e. g. the complex ester formed by reacting one mole of sebacic acid with two moles of tetraethylene glycol and two moles of 2-ethyl-hexanoic acid, complex ester formed by reacting one mole of tetraethylene glycol with two moles of sebacic acid and two moles of 2-ethyl hexanol, complex ester formed by reacting together one mole of azelaic acid, one mole of tetraethylene glycol, one mole of  $\text{C}_8$  Oxo alcohol, and one mole of  $\text{C}_8$  Oxo acid), esters of phosphoric acid (e. g. the ester formed by contacting three moles of the mono methyl ether of ethylene glycol with one mole of phosphorus oxychloride, etc.), halocarbon oils (e. g. the polymer of chlorotrifluoroethylene containing twelve recurring units of chlorotrifluoroethylene), alkyl silicates (e. g. methyl polysil-

oxanes, ethyl polysiloxanes, methyl-phenyl polysiloxanes, ethyl-phenyl polysiloxanes, etc.), sulfite esters (e. g. ester formed by reacting one mole of sulfur oxychloride with two moles of the methyl ether of ethylene glycol, etc.), carbonates (e. g. the carbonate formed by reacting C<sub>8</sub> Oxo alcohol with ethyl carbonate to form a half ester and reacting this half ester with tetraethylene glycol), mercaptals (e. g. the mercaptal formed by reacting 2-ethyl hexyl mercaptan with formaldehyde), formals (e. g. the formal formed by reacting C<sub>13</sub> Oxo alcohol with formaldehyde), polyglycol type synthetic oils (e. g. the compound formed by condensing butyl alcohol with fourteen units of propylene oxide, etc.), or mixtures of any of the above in any proportions. Mixtures of these synthetic oils and mineral oils and/or other oils described heretofore may also be employed if desired.

For the best results the base stock chosen should normally be that oil which without the new additives present gives the optimum performance in the service contemplated. However, since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additives, although in some cases auxiliary solvent agents may be used. The lubricating oils, however they may have been produced, may vary considerably in viscosity and other properties depending upon the particular use for which they are desired, but they usually range from about 34 to 150 seconds Saybolt viscosity at 210° F. For the lubrication of certain low and medium speed diesel engines the general practice has been often been to use a lubricating oil base stock prepared from naphthenic or aromatic crudes and having a Saybolt viscosity at 210° F. of 45 to 90 seconds and a viscosity index of 0 to 50. However, in certain types of diesel service, particularly with high speed diesel engines, and in aviation engine and other gasoline engine service, oils of higher viscosity index are often preferred, for example, up to 75 to 100, or even higher viscosity index.

Particularly preferred lubricating oils for automotive engines are those described in copending application Serial Number 375,158 by Leonard E. Moody and Alexander H. Popkin, filed August 19, 1953, now abandoned, which have a low "resinification index," that is, lubricating oils which have relative freedom from forming tenaciously adhering resin-like deposits when subjected to combustion in a container under a hot, smokeless flame, such as a hydrogen flame. In particular, refined mineral oil distillates obtained from paraffinic or naphthenic-base crude oils and boiling essentially within the range of about 275° to 600° F., preferably within the range of about 300° to 575° F., at 10 min. Hg absolute, are preferred base stocks.

In addition to the materials to be added to the lubricating oil base stocks according to the present invention, other agents may also be used, such as dyes, pour depressors, heat thickened fatty oils, sulfurized fatty oils, organo metallic compounds, metal phenates, metallic or other soaps, sludge dispersers, anti-oxidants, thickeners, oiliness agents, resins, rubber, olefin polymers, voltolized fatty oils or fats, voltolized mineral oils, and/or voltolized waxes and colloidal solids such as graphite or zinc oxide, etc. Solvents and assisting agents, such as esters, ketones, alcohols, aldehydes, halogenated or nitrated compounds, and the like, may also be employed.

The lubricating oil compositions of this invention comprise a major proportion of a lubricating oil base stock which, as described heretofore, include mineral oils and synthetic oils or mixtures thereof. Quite generally, the lubricating oil base stock will represent in the range of about 55 to 99.9% by weight of the total composition.

The zinc dialkyl dithiophosphates are utilized in the lubricating oil compositions in a proportion in the range of about 0.05 to 2.5% by weight based on the total composition, preferably in the range of about 0.1 to 1.5% by weight. The esters of ricinoleic acid are utilized in the lubricating oil compositions at a concentration in the range of about 0.1 to 1.5% by weight based on the total composition, preferably at a concentration in the range of about 0.2 to 0.7% by weight. The combination of the zinc dialkyl dithiophosphate and the ester of ricinoleic acid is preferably such that the weight ratio of dithiophosphate to ricinoleate is in the range of about 1:2 to 4:1, and more preferably in the range of about 1:1 to 3:1. The detergent inhibitor, which may be an alkaline earth metal alkyl phenol sulfide, an alkaline earth metal sulfonate or a mixture thereof, when included in the compositions of this invention, is utilized in general at a concentration in the range of about 0.5 to 15% by weight based on the total composition and preferably at a concentration in the range of about 1.0 to 5.0% by weight. When viscosity index improvers of the polyolefin type, such as polymerized polyisobutylene, are included in the compositions of this invention, it is generally desired to employ them at a concentration in the range of about 0.5 to 30.0% by weight, preferably about 1 to 10% by weight based on the total composition. As a general rule, viscosity index improvers of the polyester type, such as polymethacrylate esters, may be used in amounts in the range of about 0.5 to 5.0% by weight. Lubricating oil compositions containing a mixture of polyolefins and polyesters may be formulated if desired. Thus, from about 3 to 10% of polybutene and about 1 to 3% of a polyester may be used.

The invention will be more fully understood by reference to the following examples. It is pointed out, however, that the examples are given for the purpose of illustration only and are not to be construed as limiting the scope of the present invention in any way.

Various compositions formulated in accordance with this invention were evaluated in a Cadillac V-8 valve train wear test. This test is carried out in the following manner. A 1952 or 1953 Cadillac engine is assembled and operated as follows:

*First phase.*—The engine is operated with a water jacket outlet temperature of 165° F. and an oil sump temperature in the range of 190° to 200° F. under zero load conditions for two hours at the following speeds:

|    | Hours | Speed |
|----|-------|-------|
| 50 | 1/4   | 1,000 |
|    | 1/2   | 1,500 |
|    | 1/2   | 1,800 |
|    | 1/4   | 2,000 |
| 55 | 2     |       |

*Second phase.*—The engine is then operated for a number of 4-hour cycles according to the following schedule:

| 60     | Hours | Operating Conditions                                          |
|--------|-------|---------------------------------------------------------------|
| 2..... |       | 1,000 R. P. M., Zero Load, 100° F. Water Outlet Temperature.  |
| 2..... |       | Cold Water Running Through the Engine Block. Engine Shutdown. |
| 65     |       |                                                               |

The "first phase" is termed the two-hour Cadillac valve train wear test and the "first phase" plus the "second phase" when carried out for a total of 100 hours is termed the 100-hour Cadillac valve train wear test.

In each test a new filter element is employed and the initial oil charge is 6 quarts. Standard valve springs (140 lbs.) and a new cam shaft and new tappets are used in each test. Before and after each test, all of the 16 tappets and cams are measured and the average dif-

ference in overall valve lifter length is the amount of wear which has occurred. This wear is expressed in  $\text{inches} \times 10^4$ . The measurement is made after the tappets and cams have remained at a constant temperature of 75° F. for 12 hours. The tappets utilized in these valve train wear tests are made from SAE-5120 carburized steel and the camshaft is made from alloy cast iron.

The following base stocks were employed to formulate the compositions which were evaluated in the valve train wear tests:

| Base stock I:                 | Volume percent |
|-------------------------------|----------------|
| V. I. improver A <sup>1</sup> | 7.4            |
| V. I. improver B <sup>2</sup> | 2.6            |
| Lubricating oil <sup>3</sup>  | 90.0           |
|                               | 100.0          |

<sup>1</sup> An oil solution containing as the active ingredient about 20% by weight of a polyisobutylene having a Staudinger molecular weight of about 18,000.

<sup>2</sup> An oil solution containing as the active ingredient about 45% by weight of a polymerized reaction product of C<sub>8</sub> to C<sub>12</sub> alcohol esters of methacrylic acid, the polymerized reaction product having a Staudinger molecular weight of about 13,000.

<sup>3</sup> A solvent extracted and dewaxed mineral oil distillate having a viscosity of 75.7 SSU at 100° F. and a viscosity of 37.2 SSU at 210° F.

| Base stock II:                | Volume percent |
|-------------------------------|----------------|
| V. I. improver B <sup>1</sup> | 3.2            |
| Lubricating oil <sup>2</sup>  | 96.8           |
|                               | 100.0          |

<sup>1</sup> Same as used in base stock I.

<sup>2</sup> A mineral lubricating oil having an API gravity of 31.7, a pour point of 5° F., an SSU viscosity at 210° F. of about 38.8 and a viscosity index of about 102.

| Base stock III:               | Volume percent |
|-------------------------------|----------------|
| V. I. improver B <sup>1</sup> | 5.2            |
| Lubricating oil <sup>2</sup>  | 94.8           |
|                               | 100.0          |

<sup>1</sup> Same as used in base stock I.

<sup>2</sup> A mineral lubricating oil of 5W-20 grade. Base stock III has an SSU viscosity at 210° F. of 53.3 and at 100° F. of 212.5.

The following detergents were employed in the compositions evaluated in the valve train wear tests:

*Detergent A.*—This additive consisted of (1) 62.5% by weight of an oil solution containing as the active ingredient 40% by weight of an 80%-20% mixture of calcium and barium tert-octyl phenol sulfides and (2) 37.5% by weight of an oil solution containing as the active ingredient 30% by weight of calcium petroleum sulfonates.

*Detergent B.*—This additive consisted of (1) 62.5% by weight of an oil solution containing as the active ingredient 40% by weight of barium tert-octyl phenol sulfide and (2) 37.5% by weight of an oil solution containing as the active ingredient 30% by weight of calcium petroleum sulfonates.

*Detergent C.*—This additive consisted of an oil solution containing, as the active ingredient, about 30% by weight of predominantly calcium didodecylbenzene sulfonate.

*Detergent D.*—This additive consisted of an oil solution containing as the active ingredient about 40% by weight of an 80%-20% mixture of calcium and barium tert-octyl phenol sulfides.

The following additives of this invention were employed in the valve train wear tests:

*Ricinoleate.*—Polyethylene glycol di-tricinoleate (containing an average of about 9 ethylene oxide units in the glycol portion).

*Dithiophosphate conc.*—An oil solution containing as the active ingredient about 55% by weight of zinc di isohexyl dithiophosphate.

*Dithiophosphate.*—Zinc di isohexyl dithiophosphate. Another additive which was employed in several of the compositions was a P<sub>2</sub>S<sub>5</sub> treated terpene which will be designated as additive X.

## 10 EXAMPLE I

The following two lubricating oil compositions were evaluated in the 2-hour Cadillac valve train wear test:

### Composition A

| Formulation: | Volume percent |
|--------------|----------------|
| Detergent A  | 5.0            |
| Base stock I | 95.0           |
|              | 100.0          |

### Composition B

| Formulation:  | Weight percent |
|---------------|----------------|
| Composition A | 99.75          |
| Ricinoleate   | 0.25           |
|               | 100.00         |

The following results were obtained in the wear tests:

Table I

| Composition | 2-Hour Wear Test<br>(Wear in Inches $\times 10^4$ ) |               |
|-------------|-----------------------------------------------------|---------------|
|             | Average Wear                                        | Range of Wear |
| A           | 6.8                                                 | 3 to 9        |
| B           | 4.1                                                 | 1 to 7        |

It will be noted that the addition of polyethylene glycol-ditrichicinoleate to the lubricating oil composition reduced wear in the valve train of the Cadillac engines.

## EXAMPLE II

The following lubricating oil compositions were also evaluated in the 2-hour Cadillac V-8 valve train wear test:

### Composition C

| Formulation: | Volume percent |
|--------------|----------------|
| Detergent B  | 8.0            |
| Base stock I | 92.0           |
|              | 100.0          |

### Composition D

| Formulation:  | Weight percent |
|---------------|----------------|
| Composition C | 99.50          |
| Ricinoleate   | 0.50           |
|               | 100.00         |

### Composition E

| Formulation:         | Weight percent |
|----------------------|----------------|
| Composition C        | 99.50          |
| Dithiophosphate conc | 0.50           |
|                      | 100.00         |

### Composition F

| Formulation:         | Weight percent |
|----------------------|----------------|
| Composition C        | 99.50          |
| Ricinoleate          | 0.25           |
| Dithiophosphate conc | 0.25           |
|                      | 100.00         |

### Composition G

| Formulation:    | Weight percent |
|-----------------|----------------|
| Composition C   | 99.50          |
| Ricinoleate     | 0.25           |
| Dithiophosphate | 0.25           |
|                 | 100.00         |

The following results were obtained with these five lubricating oil compositions in the 2-hour Cadillac V-8 valve train wear test:

11  
Table II

| Composition | 2-Hour Test<br>(Wear in Inches $\times 10^4$ ) |               |
|-------------|------------------------------------------------|---------------|
|             | Average Wear                                   | Range of Wear |
| C           | 6.3                                            | 3 to 11       |
| D           | 6.0                                            | 4 to 10       |
| E           | 12.0                                           | 5 to 18       |
| F           | 4.4                                            | 3 to 6        |
| G           | 2.2                                            | 0 to 5        |

It will be noted that the combination of the ricinoleate and zinc di isohexyl dithiophosphate (compositions F and G) demonstrated synergism. Thus the combination was better than either the ricinoleate (composition D) or the dithiophosphate (composition E) when these additives were employed separately.

## EXAMPLE III

The following two lubricating oil compositions were evaluated in the 100-hour Cadillac V-8 valve train wear test:

Composition H

| Formulation:  | Volume percent |
|---------------|----------------|
| Detergent B   | 8.0            |
| Base stock II | 92.0           |
|               | 100.0          |

Composition I

| Detergent B          | 8.00   |
|----------------------|--------|
| Ricinoleate          | 0.13   |
| Dithiophosphate conc | 0.26   |
| Base stock II        | 91.61  |
|                      | 100.00 |

These two lubricating oil compositions gave the following results in a 100-hour Cadillac V-8 valve train wear test:

Table III

| Composition | 100-Hour Test<br>(Wear in Inches $\times 10^4$ ) |               |
|-------------|--------------------------------------------------|---------------|
|             | Average Wear                                     | Range of Wear |
| H           | 15.4                                             | 7 to 33       |
| I           | 12                                               | 7 to 19       |

It will be noted again that the addition of a combination of polyethylene glycol-di-trricinoleate and a zinc dialkyl dithiophosphate substantially reduced valve train wear in Cadillac engines.

## EXAMPLE IV

The following two lubricating oil compositions were also evaluated in the 100-hour Cadillac V-8 valve train wear test:

Composition J

| Formulation:                  | Volume percent |
|-------------------------------|----------------|
| Additive mixture <sup>1</sup> | 8.5            |
| Base stock III                | 91.5           |
|                               | 100.0          |

<sup>1</sup> Detergent C  
Detergent D  
Dithiophosphate concentrate  
Additive X

100.0

12  
Composition K

| Formulation:                  | Volume percent |
|-------------------------------|----------------|
| Additive mixture <sup>1</sup> | 8.5            |
| Ricinoleate                   | 0.5            |
| Base stock III                | 91.0           |
|                               | 100.0          |

<sup>1</sup> Same as used in composition J.

Table IV

| Composition | 100-Hour Test<br>(Wear in Inches $\times 10^4$ ) |               |
|-------------|--------------------------------------------------|---------------|
|             | Average Wear                                     | Range of Wear |
| J           | 23                                               | 6 to 46       |
| K           | 10.5                                             | 7 to 15       |

It will be noted again that the combination of polyethylene glycol-di-trricinoleate and zinc dialkyl dithiophosphate substantially reduced valve train wear in Cadillac engines.

## EXAMPLE V

The following two lubricating oil compositions were also evaluated in the 100-hour Cadillac V-8 valve train wear test:

Composition L

| Formulation:         | Volume percent |
|----------------------|----------------|
| Detergent C          | 3.55           |
| Detergent D          | 2.13           |
| Dithiophosphate conc | 0.89           |
| Additive X           | 0.53           |
| Base stock I         | 92.90          |
|                      | 100.00         |

Composition M

| Detergent C          | 3.55   |
|----------------------|--------|
| Detergent D          | 1.88   |
| Dithiophosphate conc | 0.89   |
| Ricinoleate          | 0.25   |
| Additive X           | 0.53   |
| Base stock I         | 92.90  |
|                      | 100.00 |

The following results were obtained in the 100-hour Cadillac V-8 valve train wear test:

Table V

| Composition | 100-Hour Test<br>(Wear in Inches $\times 10^4$ ) |               |
|-------------|--------------------------------------------------|---------------|
|             | Average Wear                                     | Range of Wear |
| L           | 18                                               | 10 to 25      |
| M           | 8                                                | 5 to 17       |

It will be noted again that the combination of polyethylene glycol-di-trricinoleate and zinc dialkyl dithiophosphate was exceedingly effective in reducing valve train wear in Cadillac engines.

What is claimed is:

1. A lubricating composition comprising a major proportion of a mineral lubricating oil, in the range of 0.1 to 1.5 wt. percent of a zinc dialkyl dithiophosphate having in the range of 8 to 16 carbon atoms per molecule, and in the range of 0.2 to 0.7 wt. percent of a polyricinoleic acid ester of a polyethylene glycol, said glycol having a molecular weight in the range of 200 to 800 and said ester being formed from a polyricinoleic acid

**13**

containing in the range of 2 to 4 molecules of self-esterified ricinoleic acid.

2. The composition of claim 1 comprising, in addition thereto, in the range of 0.5 to 15 wt. percent of a detergent selected from the group consisting of alkaline earth metal alkyl phenol sulfides and alkaline earth metal sulfonates.

3. A lubricating composition comprising a major proportion of a mineral lubricating oil, in the range of 0.1 to 1.5 wt. percent of zinc diisohexyl dithiophosphate, 10 and in the range of 0.2 to 0.7 wt. percent of polyethylene di-triricinoleate containing an average of about 9 ethylene oxide units in the glycol portion.

4. A lubricating composition comprising a major pro-

**14**

portion of a mineral lubricating oil, about 0.89 wt. percent of a 55 wt. percent concentration in oil of zinc diisohexyl dithiophosphate, and 0.25 wt. percent of polyethylene glycol di-triricinoleate containing an average of about 9 ethylene oxide units in the glycol portion.

**References Cited in the file of this patent**

**UNITED STATES PATENTS**

|           |             |       |               |
|-----------|-------------|-------|---------------|
| 2,210,140 | Colbeth     | ----- | Aug. 6, 1940  |
| 2,364,283 | Freuler     | ----- | Dec. 5, 1944  |
| 2,457,139 | Fife et al. | ----- | Dec. 28, 1948 |
| 2,506,310 | Mikeska     | ----- | May 2, 1950   |

UNITED STATES PATENT OFFICE  
CERTIFICATE OF CORRECTION

Patent No. 2,824,836      Harlan M. Smith et al.      February 25, 1958

It is hereby certified that error appears in the printed specification of the above numbered patent requiring correction and that the said Letters Patent should read as corrected below.

Column 13, line 11, after "polyethylene" insert -- glycol --.

Signed and sealed this 17th day of June 1958.

(SEAL)

Attest:

KARL H. AXLINE

Attesting Officer

ROBERT C. WATSON  
Commissioner of Patents